

July 4, 1972

YOO IIJIMA ET AL

3,674,491

DEVELOPING PROCESS

Filed Nov. 30, 1970

FIG. 1



FIG. 2



FIG. 3



INVENTORS  
YOO IIJIMA  
ISAO SHIMAMURA  
TOKIHARU KONDO  
HARUHIKE IWANO

BY *Sagrove, Rothwell, Mun,  
Zum & Macpeak*

ATTORNEYS

1

3,674,491

## DEVELOPING PROCESS

Yoo Iijima, Isao Shimamura, Tokiharu Kondo, and Haru-hiko Iwano, Kanagawa, Japan, assignors to Fuji Photo Film Co., Ltd., Kanagawa, Japan

Filed Nov. 30, 1970, Ser. No. 93,672

Claims priority, application Japan, Nov. 29, 1969,  
44/95,485  
Int. Cl. G03c 5/30

U.S. Cl. 96—66.3

16 Claims

### ABSTRACT OF THE DISCLOSURE

A process for developing a silver halide photographic light-sensitive material which comprises developing the light-sensitive material in the presence of a compound represented by the following general formula:



wherein R represents an unsubstituted or substituted alkyl group of 1-5 carbon atoms, aralkyl group of 1-5 carbon atoms, or aryl group, and R<sub>1</sub> and R<sub>2</sub> each represents a hydrogen atom or an alkyl group of 1-5 carbon atoms, said R<sub>1</sub> and R<sub>2</sub> also capable of forming an unsaturated condensed ring of 5-6 carbon atoms, which may be further substituted by an alkyl group of 1-5 carbon atoms.

### BACKGROUND OF THE INVENTION

#### Field of the invention

The present invention relates to a process for developing silver halide photographic light-sensitive materials and more particularly to a development process for reducing the gamma of a photographic image.

#### Description of the prior art

It is very important to control the gradation of the gamma of an image obtained when developing with a silver halide photographic material. It is also important to reduce the grain size of the developed silver particles. Various types of fine grain developing solutions have been known. For instance, some of them are disclosed in the specifications of U.S. Pats. Nos. 2,113,312; 2,164,280; 2,311,428 and 2,840,471 and the specification of British Pat. No. 723,286. However, the resolving power and granularity of the images obtained by these known fine-grain developers still remain insufficient for micro-filming insofar as ordinary photographic films or papers, which are not designed for micro-filming, are concerned. A light-sensitive material for micro-filming is commercially available as a material having a high resolving power and good granularity. Although this material has excellent resolving power and granularity, the gamma of the processed image is too high for recording of tonal scenery.

Therefore, it would be quite profitable to develop a method for obtaining a micro-image having soft gradation, high resolving power and reduced granularity by employing a micro-film which gives hard tone with conventional development. Various investigations have been conducted for finding such a developing process suitable for such purposes. In this regard, there is known, for example, French Pat. No. 1,495,935. In this patent, the soft tone is obtained by pre-treating a photographic film with an aqueous solution of a noble metal salt before development. In Japanese patent publication No. 14,510/69 (Japanese Pat. No. 561,153), the image tone of a high gamma photographic film is softened by developing it by a conventional soft tone developing solution and fixing

2

the film with a fixing solution containing an oxidizing agent. This procedure, however, has the shortcoming of a decreased fixing rate.

In this process, the fixing time must be strictly controlled and the life of fixing solution is reduced, since the fixer contains an oxidizing agent, which makes the treatment of the process difficult. On the other hand, in the process of the French Pat. No. 1,495,935, an inexpensive noble metal is used and an additional processing step is required, which makes the developing process complicated. Hence, it is very difficult to obtain a soft tone image using a high gamma photographic film by only employing the device in a conventional development procedure.

Furthermore, a developing solution containing 1-phenyl-3-pyrazolidone as the sole developing agent can be used in order to reduce the gamma of the image but it is accompanied by low sensitivity. In addition, it is very easily exhausted by processing small quantities of films. On the other hand, a developing solution containing N-methyl-p-aminophenol may have a high sensitivity but it is not effective for obtaining a soft tone image. Moreover, a developing solution combining suitable amounts of 1-phenyl-3-pyrazolidone and N-methyl-p-aminophenol may exhibit high sensitivity and provide a considerably soft tone image but is easily exhausted. Furthermore, a developing solution containing a proper amount of 1-phenyl-3-pyrazolidone, N-methyl-p-aminophenol and hydroquinone may have a high sensitivity and is not easily exhausted but it is impossible to obtain good soft tone images by using such a developing solution.

As mentioned above, many attempts have been made to solve the problem but none has every fully satisfied the requirements for recording tonal objects on a microfilm or paper. That is, they never provide sufficient sensitivity for printing work, gradation soft enough for recording the tonal scenery, or good resistivity to exhaustion.

### SUMMARY OF THE INVENTION

It is, therefore, the primary object of the present invention to provide a process for producing soft tone images without any loss of granularity and resolving power by using silver halide photographic recording materials of fine grain, high contrast and relatively low sensitive type.

Accordingly, the object of this invention can be achieved by developing high contrast silver halide photographic light-sensitive material in the presence of a compound represented by the following formula:



wherein R represents an unsubstituted or substituted \* alkyl group of 1-5 carbon atoms, aralkyl group of 1-5 carbon atoms or aryl group and R<sub>1</sub> and R<sub>2</sub> each represents a hydrogen atom or an alkyl group of 1-5 carbon atoms, said R<sub>1</sub> and R<sub>2</sub> also capable of forming an unsaturated condensed ring of 5-6 carbon atoms, which may be further substituted by an alkyl group of 1-5 carbon atoms.

Illustrative of the compounds shown above to be employed in the present invention follow,

\*Any substituent will suffice, providing however, it does not detract from the goals of the present invention.

| Compound | M.P., °C. |
|----------|-----------|
| 1.       | 153-154   |
| 2.       | 126-127   |
| 3.       | 131-132   |
| 4.       | 151-152   |
| 5.       | 128-129   |
| 6.       | 145-146   |
| 7.       | 193-194   |

These compounds may be synthesized generally by the following process:

#### DETAILED DESCRIPTION OF THE INVENTION

##### Synthesis example

Synthesis of 2 - (S - ethylglycolamido)benzothiazole (Compound 5)—34 g. of 2-aminobenzothiazole was dissolved in 120 ml. of anhydrous pyridine. Subsequently, an ether solution of 38.5 g. of chloroacetyl chloride was added dropwise to the solution with stirring while cooling the solution to temperatures lower than  $-5^{\circ}\text{C}$ . Thereafter, the mixture was further stirred for 2 hours at room temperature to complete the reaction. Then the solution was poured into 2 liters of water and the precipitated crystals were recovered. 36 g. of crude 2-chloroacetamido-benzothiazole having a melting point of 160-163° C., was obtained.

2.8 g. of potassium hydroxide was dissolved into about 70 ml. of ethanol. After adding to the solution 11.32 g. of 2-chloroacetamido-benzothiazole, as prepared above, the mixture was refluxed for 4 hours under heating. The reaction product was concentrated under a reduced pressure and dried. The product was then extracted with benzene. After distilling the benzene away, the residue was recrystallized from 50% alcohol to give 5 g. of 2-(S-ethylglycolamido)benzothiazole having a melting point of 128-129° C.

By following the same procedure as illustrated above using methyl mercaptan instead of ethyl mercaptan, 2-(S-methylthioglycolamido)benzothiazole (Compound 4) was obtained. Also, by using thiophenol instead of ethyl mercaptan in the above procedure, 2-(S-phenylthioglycolamido)benzothiazole (Compound 6) was obtained. Furthermore, by using 2-aminothiazole instead of 2-amino-benzothiazole, the corresponding thiazole derivatives (Compounds 1-3) were obtained. Also, by using 2-amino-5-methyl-benzothiazole instead of 2-amino-benzothiazole

in the above procedure, 2-(S-methylthioglycolamido)-5-methyl-benzothiazole (Compound 7) was obtained.

The compounds of this invention can be applied to generally high contrast silver halide photographic recording materials of fine grain and relatively low sensitivity.

Various organic anti-foggants, such as 6-nitrobenzimidazole, benzotriazole, or 1 - phenyl-5-mercaptopterazole 45 are known. The addition of large amounts of such compounds to the developer will also lower the gamma, but since the sensitivity is greatly reduced, the use of the compounds for this purpose is not practicable.

The addition of a large amount of other developing 50 inhibitors, such as potassium bromide or potassium iodide, will also lower the gamma, but these compounds are impracticable for the same reason as indicated above.

The developing solution containing the above compound of the present invention contains at least one developing agent, such as hydroquinone, 1-phenyl-3-pyrazolidone, N - methyl-p-amino-phenol, etc. Furthermore, it contain one or more antioxidants, such as sodium sulfite, ascorbic acid, etc.; a salt such as sodium sulfate, a pH adjusting agent and a buffering agent, such as boric acid, borax, sodium hydroxide, sodium carbonate and sodium phosphate, and the like.

In order to enhance the softening, potassium bromide or potassium iodide may be used together with the compound of this invention. Further, for reducing the formation 65 of fogs, other organic anti-foggants may be used together with the compounds of the present invention. In some cases, an aldehyde such as formalin or glutaraldehyde or an organic solvent such as triethylene glycol and hexylene glycol may be added. Still further, a developing accelerator such as an amine or a polyethylene glycol may also be used together with the compounds of this invention.

In case of adding the compound of this invention to a 70 developing solution, the amount of the compound added



The photographic properties of the images thus obtained are shown in the following table:

| Developing solution | Compound (amount)      | Photographic property |       |
|---------------------|------------------------|-----------------------|-------|
|                     |                        | Fog                   | Gamma |
| D                   |                        | 0.11                  | 1.08  |
| J                   | Compound 6 (50 mg./l.) | 0.10                  | 0.68  |
| K                   | Compound 7 (50 mg./l.) | 0.10                  | 0.65  |

As indicated in the results above, soft tone development could be attained by the addition of the Compounds 6 or 7 of this invention.

#### EXAMPLE 4

A microfilm prepared by coating a support with a fine grain silver chlorobromide gelatin emulsion was exposed by means of a sensitometer and developed by developing solution L of this invention at 27° C.

For the sake of comparison, the same developing procedure was followed using the developing solution M having the same composition as the developing solution L, except that it did not contain the Compound 2 of this invention.

#### Developing Solution L:

|                                  |      |     |
|----------------------------------|------|-----|
| N-methyl-p-aminophenol sulfate   | g--  | 8.0 |
| sodium sulfite                   | g--  | 125 |
| sodium carbonate mono-hydrate    | g--  | 6.7 |
| Potassium bromide                | g--  | 2.5 |
| Compound 2                       | mg-- | 50  |
| Water added to make, to 1 liter. |      |     |

The photographic properties of the images thus obtained are shown in the following table:

| Developing solution | Added compound (addition amount) | Photographic property |       |
|---------------------|----------------------------------|-----------------------|-------|
|                     |                                  | Fog                   | Gamma |
| L                   | Compound 2 (50 ml./l.)           | 0.11                  | 0.67  |
| M                   |                                  | 0.13                  | 1.42  |

#### EXAMPLE 5

A microfilm prepared by coating a support with a fine grain silver chlorobromide gelatin emulsion was exposed by means of a sensitometer and then developed by the developing solution N having the following composition of this invention.

For the sake of comparison, the same developing procedure was followed using a comparison developer O having the same composition as that of the developing solution M mentioned in Example 4 from which the Compound 5 of this invention had been omitted.

#### Developing Solution N:

|                                                  |      |     |
|--------------------------------------------------|------|-----|
| 1-phenyl-3-pyrazolidone                          | g--  | 4.0 |
| N-methyl-p-aminophenol sulfate                   | g--  | 2.0 |
| Sodium sulfite                                   | g--  | 100 |
| Sodium carbonate mono-hydrate                    | g--  | 30  |
| Hydroquinone                                     | g--  | 2.0 |
| Potassium bromide                                | g--  | 5.0 |
| Compound 5                                       | mg-- | 50  |
| Water added to make the whole volume to 1 liter. |      |     |

The photographic properties of the images obtained by the development are shown in the following table:

| Developing solution | Compound (amount)       | Photographic property |       |
|---------------------|-------------------------|-----------------------|-------|
|                     |                         | Fog                   | Gamma |
| N                   | Compound 5 (100 mg./l.) | 0.10                  | 0.66  |
| O                   |                         | 0.12                  | 1.38  |

A 1-phenyl-3-pyrazolidone/N-methyl-p-aminophenol/hydroquinone type developing solution has a higher processing function than a 1-phenyl-3-pyrazolidone/N-methyl-p-aminophenol type developing solution but shows undesirably high gamma characteristics. However, by adding

75

the Compound 5 of this invention to the former type developing solution, soft tone developments can be attained. Furthermore, the developing power becomes higher, as shown in the above table.

When all of those compounds disclosed in col. 3 of the present application are substituted with methyl or ethyl radicals as in Compound 7, identical and even better results (in some cases) are observed.

Although the present invention has been adequately described in the foregoing specification and examples included therein, it is readily apparent that various modifications and changes may be made without departing from the intended scope thereof.

What is claimed is:

1. A process for developing a silver halide photographic light-sensitive material which comprises developing the light-sensitive material in the presence of a compound represented by the following general formula:



wherein R represents an unsubstituted or substituted alkyl group of 1-5 carbon atoms, aralkyl group of 1-5 carbon atoms, or aryl group, and R<sub>1</sub> and R<sub>2</sub> each represents a hydrogen atom or an alkyl group of 1-5 carbon atoms, said R<sub>1</sub> and R<sub>2</sub> also capable of forming an unsaturated condensed ring of 5-6 carbon atoms, which may be further substituted by an alkyl group of 1-5 carbon atoms.

2. The process of claim 1 wherein said compound is contained in a developer.

3. The process of claim 2 wherein said developer is a developer for forming soft tone images on microfilm.

4. The process of claim 1 wherein said compound is:



5. The process of claim 1 wherein said compound is:



6. The process of claim 1 wherein said compound is:



7. The process of claim 1 wherein said compound is:



8. The process of claim 1 wherein said compound is:



9. The process of claim 1 wherein said compound is:



10. The process of claim 1 wherein said compound is:



11. The process of claim 2 wherein the concentration of said compound ranges from 1 mg.-10 g. per liter of developing solution.

12. The process of claim 11 wherein the concentration of said compound ranges from 30-100 mg. per liter of 5 developing solution.

13. The process of claim 1 wherein a photographic emulsion containing said compound is employed.

14. The process of claim 13 wherein the concentration of said compound in said emulsion ranges from 1 mg.- 10 10 g. per kg. of emulsion.

15. The process of claim 14 wherein the concentration of said compound ranges from 50-200 mg./kg. of emulsion.

16. The silver halide photographic light-sensitive mate- 15 rial developed by the process of claim 1.

## UNITED STATES PATENTS

|           |        |                      |         |
|-----------|--------|----------------------|---------|
| 3,046,130 | 7/1962 | Dersch et al. -----  | 96—66.3 |
| 3,084,044 | 4/1963 | Dersch et al. -----  | 96—66.3 |
| 3,342,596 | 9/1967 | Graham -----         | 96—66.3 |
| 3,502,467 | 3/1970 | Becker -----         | 96—66.3 |
| 3,305,362 | 2/1967 | Riester et al. ----- | 96—66   |

NORMAN G. TORCHIN, Primary Examiner

E. C. KIMLIN, Assistant Examiner

U.S. CL. X.R.

96—66, 95